

# UNITED STATES PATENT OFFICE.

BENNO BORZYKOWSKI, OF CHARLOTTENBURG-BERLIN, GERMANY.

PRODUCTION OF ARTICLES OR MATERIALS FROM VISCOSE.

Specification of Letters Patent.

Application filed May 17, 1913. Serial No. 768,282.  
Patented June 15, 1915.

1,143,569.

No Drawing.

To all whom it may concern:

Be it known that I, BENNO BORZYKOWSKI, a subject of the Russian Emperor, residing at Neue Kantstrasse 1, Charlottenburg-Berlin, Germany, have invented certain new and useful Improvements in the Production of Articles or Materials from Viscose; and I do hereby declare the following to be a full, clear, and exact description of the invention, such as will enable others skilled in the art to which it appertains to make and use the same.

According to the known processes, viscose is obtained in stable form, as threads, films and the like, by means of acid solutions or solutions of mineral salts. The products are, however, imperfect, and do not fulfil all requirements. They generally become cloudy in course of time, or brittle and lose their luster and can no longer be evenly dyed, which is caused by the products of decomposition of cellulosexanthogenate, with simultaneous deposit of sulfur in the interior of the threads. Attempts have been made to overcome these drawbacks by adding to the ordinary precipitating baths, higher alcohols, such as glucose or fatty acids in considerable quantities, or by treating the artificial products at a later stage with salts having an affinity for sulfur.

The present invention depends, in principle, upon the surprising observation that by adding organic "nitroso" bases, such for instance as p-nitroso-dimethyl-anilin, or p-nitroso-diethyl-anilin or the like, or their salts, to the precipitating bath, such for instance as alkaline chlorids, sulfates and the like, in neutral or acid solutions, very valuable properties, from a technical point of view, are given to the articles to be produced. Even a small addition of the nitroso bodies to the cold or warm precipitating baths prevents the decomposition of the cellulosexanthogenate with the consequent deposition of free sulfur, since it protects it from oxidation, and the article, for instance a thread, film or the like, obtained from a precipitating bath, is distinguished even in the wet and raw state by a great amount of luster, great transparency and great stability.

When spinning the viscose, it can be wound upon spools or reels in the form of threads, immediately after leaving a circulating precipitating bath constituted as above described. The reels or spools are

then rotated in a weak alkaline finishing bath, for instance one containing sodium sulfid. In this way the removal of the sulfur is effected, and at the same time the above named bases separate out from the solution on to the outer surface of the thread and are there reduced to amido bases, for instance p-amido-dimethyl-anilin, or p-amido-diethyl-anilin, or in any case the nitroso compound corresponding to the protective coating. At the same time, they prevent the capillary threads sticking together so that a yarn of fine silky texture is obtained. By subsequent treatment with weak acids, cellulose hydrate is obtained, and at the same time the amido bases go into solution to form salts. These latter, after the acid baths have become sufficiently rich, can be recovered and form valuable by-products.

The articles obtained by this process from viscose are remarkable for their great brilliancy and strength, and they also have a clear color and are unusually stable and elastic. This makes the substance adaptable for use for all textile purposes, especially for weaving, for instance in the form of near silk, as the material can be used only for forming the weft but also for the warp, and fulfills all requirements on account of its great strength and facility of drawing. The finished articles or materials not change their properties or appearance when exposed to the air, and they can evenly dyed. They are perfectly stable. The composition of the precipitating bath may of course vary considerably.

The following example illustrates the process:—The precipitating bath consists of sodium chlorid in 100 parts of water, 15 parts of sodium chlorid, 10 parts of ammonium sulfate and .5 parts of p-nitroso-dimethyl-anilin, the last mentioned being previously dissolved in sulfuric acid. The threads pass to a spool rotating in a solution to 60° or 70° C. of 10 parts of ammonium sulfate and .5 parts sodium sulfide in 100 parts of water, the spool being kept at a suitable speed. It will be understood that all proportions in this example are stated by weight.

From the precipitating or settling threads may be passed through a guide device, to winding reels, v

ing reels also rotate in the alkaline solution, after which the finished thread may be dealt with in the form of skeins.

It may finally be stated that it is possible for obtaining technically valuable results with the present process to employ every kind of viscose solution in all liquid states of their maturation both raw and cleaned.

The expression "nitroso bases" as used in the appended claims refers to these bases, whether in the free state, or combined with an acid, to form salt of the bases.

What I claim and desire to secure by Letters Patent of the United States of America is:—

1. A process of producing articles from viscose, which comprises subjecting a viscose solution to the action of a setting bath, said bath containing an organic nitroso base.
2. A process of producing articles from viscose which comprises subjecting viscose solution to a setting bath containing an organic nitroso base, and thereafter immediately treating the precipitated viscose with a weak alkaline solution.

3. A process of producing articles from viscose which comprises subjecting said viscose in solution to the action of a setting bath containing a p-nitroso-anilin derivative.

4. A process of producing articles from viscose, which comprises subjecting said viscose in solution to the action of a setting bath containing an organic nitroso base, then subjecting the precipitated viscose to the action of a weak alkaline solution, and thereafter subjecting said viscose to the action of a weak acid.

5. A process of setting viscose which comprises subjecting said viscose in solution to the action of a bath containing 100 parts of water, 15 parts of sodium chloride, 10 parts of ammonium sulfate, and .5 parts of p-nitroso-dimethyl-anilin.

In testimony whereof, I affix my signature, in presence of two witnesses.

BENNO BORZYKOWSKI.

Witnesses:

WOLDEMAR HAUPT,  
HENRY HASPER.